

Jan. 9, 1934.

E. D. REYNOLDS

1,942,451

WOVEN WIRE AND METHOD OF PRODUCING THE SAME

Filed Feb. 26, 1930

Fig. 1



Fig. 2.



Fig. 3.



Inventor:

Elmer D. Reynolds

By

Wilson, Dowell, McCausa + Rehm

Attest.

## UNITED STATES PATENT OFFICE

1,942,451

WOVEN WIRE AND METHOD OF PRODUC-  
ING THE SAME

Elmer D. Reynolds, Dixon, Ill., assignor to Reynolds Wire Co., Dixon, Ill., a corporation of Illinois

Application February 26, 1930. Serial No. 431,631

9 Claims. (Cl. 29—148)

My invention relates to wire cloth and has special reference to wide-mesh cloth wherein the wire employed in its manufacture is relatively fine or small in diameter.

In the past it has been necessary to manufacture wide-mesh cloth, for example, 2 to 10 mesh cloth, from relatively heavy wire, usually .02 of an inch in diameter or greater. By 2 to 10 mesh cloth I mean cloth having 2 to 10 strands per inch. There are a great many uses to which wide-mesh cloth may be put wherein a heavy wire is not necessary and wherein the cost of such a cloth becomes prohibitive. Among such uses may be mentioned those wherein wire cloth is placed between layers of paper, cloth, felt, or the like, or other materials of low mechanical strength for the purposes of reenforcement. In many cases heavy wire cloth is a positive detriment because of the reduction in the flexibility of the sheet resulting from its use. Fine wire wide-mesh cloth, while considerably cheaper, because of the smaller amount of metal required in its manufacture, has been so unstable that it collapses during handling and before it can be positioned between the sheets or imbedded in the sheet material with which it is to be used, and consequently has not been available commercially. However, after the cloth is positioned it is usually suitably held between the sheets or the like by adhesives whereby it is prevented from collapsing. The problem therefore, is to provide a metal cloth of this character at low cost having sufficient stability to withstand the abuse incident to its handling between the time of its manufacture and the time when it is finally positioned in the material with which it is to be used. When finer wire has been used it has been very difficult to maintain the strands in their proper position, the strands spontaneously moving out of position, distorting the cloth sheet and rendering it practically valueless. As a matter of fact, when the wire becomes too small, the strands move to such an extent under the natural spring tension placed upon them during weaving, that the cloth collapses, becoming a mere mass of tangled wire.

A portion of the trouble doubtless arises from the character of the wire employed. Most wire, such as of brass, copper, steel, and the alloys of steel, used for the manufacture of wire cloth, is cold-drawn, and as a result of the drawing operations it is hardened and given a certain springiness. When such wire is woven it is bent to the desired position to form the cloth. These bending operations set up strains in the metal which

result in a tendency for the wire to return to its prior condition. However, when fine wire is used for a wide-mesh cloth very little, if any, crimp is formed in the wire. This is, of course, necessarily so, since, as the diameter of the wire increases and the width of the mesh increases, the size of the angle through which the wire must be bent to pass over one strand and under another, decreases. In reality when wire such as that contemplated in my invention is employed to form woven cloth, the individual strands are practically straight, and have no appreciable crimp. It is this crimp or bend in the wire which normally causes the individual strands of the woven cloth to maintain their position, against the spring tension of the wire, and thus lend permanent structure to the cloth. The absence of this crimp and the decrease in the rigidity of the wire itself, aided by the tension under which the wire is placed by weaving, results in the cloth having a tendency to collapse, as set forth. For these reasons it has been, if not impossible, highly impractical to manufacture satisfactory cloth of this character.

I have therefore aimed to provide a method for manufacturing wide-mesh wire cloth at a lower cost than has heretofore been possible.

Another object of the invention is the provision of a method for manufacturing wide-mesh cloth wherein wire of substantially smaller diameter may be employed to produce a commercially usable product at a substantial reduction in material cost.

Another object of the invention is the provision of a wide-mesh cloth of a smaller wire than has heretofore been possible.

A still further object of the invention is the provision of a woven wide-mesh wire cloth wherein the individual strands are of small diameter and are held in position solely because of their weaving and require no additional means for stabilizing the cloth.

Other objects and attendant advantages will become apparent to those skilled in the art from the following description and the accompanying drawing, in which

Figure 1 is a diagrammatic view showing the manner in which the woven cloth emerges from the loom and is wound into rolls;

Fig. 2 is a diagrammatic view showing a cross-section of an oven with the rolls of cloth positioned on end therein for treatment; and

Fig. 3 is a perspective view of a completed roll of cloth showing the manner in which the cloth

105

110

may be unrolled to lie flat after it has been heat-treated.

Heretofore it has been impractical to manufacture wire screen cloth of less than twelve-mesh 5 of wire having a diameter less than .02 of an inch. In commercial practice it has been found that the use of smaller wire results in a perishable product which cannot be satisfactorily stored or handled. The usual practice is to make no 10 cloth of less than twelve-mesh of wire having a diameter less than .02 of an inch. However, cloth down to six-mesh may be made of wire having this diameter. Five-mesh cloth is made of wire not smaller than .023, four-mesh cloth of wire not 15 smaller than .028, three-mesh cloth of wire not smaller than .032, and two-mesh cloth of wire not smaller than .041.

In carrying out my invention I employ wire of diameter substantially smaller than the smallest heretofore considered practical. For example, 20 in commercial practice I have satisfactorily used wire of .01 of an inch in diameter for the manufacture of four-mesh cloth. This fine wire may be used in the manufacture of cloth of 12-mesh or less which may be stored and handled without material depreciation. The invention is particularly advantageous, however, in the manufacture 25 of cloth of less than six-mesh, for as the mesh decreases below this point it has been necessary in the past to increase the diameter of the wire as previously set forth. I have found the invention of particular value in the manufacture 30 of reinforcing cloth of four-mesh for which I have satisfactorily employed wire of a diameter 35 of .01 of an inch.

According to my invention the wire to be used in the manufacture of fine wire wide-mesh cloth is made by any of the usual wire-drawing processes. The cold drawing processes produce a wire 40 which is hardened and has a considerable amount of springiness, such as cold drawn steel wire. While the hardness produced in wires of this character is a desirable characteristic, the spring 45 tendency of the wire becomes a problem in the manufacture of cloth of this type. The wire is woven into cloth in the usual manner on the usual wire cloth loom, the numeral 6 designating the cloth as it comes from a loom indicated by the dotted lines bearing the numeral 7 in Fig. 1. 50 These looms continuously wind up the cloth, as it is being woven, into rolls 9 of desired size around center pieces indicated generally by the numeral 8. When the rolls contain several hundred feet 55 of the cloth they are tied up tightly and removed bodily from the loom, the center piece 8 being removed therefrom. The rolls as they are removed from the loom are taken to a heat treating oven 11, as shown in Fig. 2, where they are placed on end and there exposed to a temperature 60 of approximately 700° F. for about two hours. I have found that any temperature in the so-called bluing range, or the range of temperature in which a blue color is conferred upon the steel, is well suited to bring about the desired results. 65 The period of time for which the heating must be continued will, of course, depend upon the temperature to which the wire is exposed, temperatures at the lower side of the bluing range requiring more time than the temperatures at the 70 upper edge of this range. Obviously also, the heating time will depend upon the quantity of wire being treated and on the time required to bring the total mass to the bluing temperature. I have found, however, that if the temperature 75 is maintained at about 700° F., about two hours

will be required to bring about the desired results.

I am led to believe that through the heating operation the strains which had previously been set up in the individual wires of the metal cloth by the drawing and weaving operations, are relieved, thereby destroying any tendency which the wires may have to move from their appointed places in the cloth. It is possible that a portion of the springiness is removed from the wire during this process, but this has been found to be insufficient to affect the strength of the cloth, if it does occur.

I have found that if the rolls, as they are removed from the loom, are permitted to stand, without this heating step, a gradual but continuous movement of the wires or individual strands of the cloth occurs spontaneously, resulting in the gradual collapsing of the cloth. On the other hand, if the wire as it comes from the loom is immediately placed in the treating oven and subjected to the heat treatment outlined, the cloth, after being removed from the oven, may be permitted to stand for an indefinite length of time without any evidence of a spontaneous collapsing. The roll may be unrolled as shown in Fig. 3 and 100 the cloth spread out in sheets 12 and handled in the usual manner without undergoing appreciable disintegration. This is in exact contrast with the untreated cloth, which, if unrolled and spread out in sheet form, tends to curl up from 105 all edges toward the center and becomes practically impossible to handle in the usual way.

Thus, the hard steel wires are bent into the desired shape in the loom. They still possess, because of the internal strain set up by this bending process, a tendency to return to their former shape. If the cloth is permitted to stand at this time the wires will gradually return, at least partially, to their previous condition, distorting the cloth and causing it to collapse. However, when 110 the cloth is subjected to heat in the oven, the strains are removed from the wires while the cloth is yet firmly held in the roll and the tendency for the individual wires to return to their previous condition is destroyed. After this operation has occurred the wires of the cloth tend to remain in the desired position and may only be moved therefrom by actual mechanical force. Even when so moved they have a slight tendency 115 to return to their desired position in the wire 120 cloth fabric.

It will be seen that by my improved process I have produced a wire cloth of wide mesh and fine strands which may be handled in every way as the ordinary wire cloth. The cloth may be unrolled and handled in the usual manner. It may be positioned in materials of low mechanical strength to produce an article of substantially lower cost than heretofore possible. It may be cut into sheets and placed between sheets of 130 cloth, rubber, or the like, without material difficulty. Because of the wide mesh and the small size of the wire, only a small amount of metal is used to make a large amount of cloth. There is, therefore, a substantial saving in the cost of 135 materials, which is reflected in a cloth of low cost. The method is simple and involves no operations directed toward tying the individual strands together other than the weaving operations themselves.

While I have thus described and illustrated a specific embodiment of my invention I am aware that numerous alterations and changes may be made therein without departing from the spirit of the invention, and I do not wish to be limited 140 145 150

except as required by the prior art and the scope of the appended claims in which—

I claim:

- 5 1. The method of making wire cloth which includes weaving wire of a diameter less than .02 of an inch into cloth of less than 12 mesh, and heating the cloth to a temperature within the bluing range of steel for a sufficient length of time to substantially relieve the strains in the wire. 80
- 10 2. The method of making wire cloth which includes weaving ferrous wire of a diameter less than .02 of an inch into cloth of less than 12 mesh, and heating the cloth to a temperature in the region of 700° F. for a time sufficient to substantially relieve the strains in the wire. 85
- 15 3. The method of making wire cloth which includes weaving ferrous wire of a diameter less than .02 of an inch into cloth of less than 12 mesh, and heating the cloth to a temperature in the region of 700° F. for about two hours. 90
- 20 4. The method of making wire cloth which includes weaving ferrous wire of a diameter less than .02 of an inch into cloth of about 4 mesh, and heating the cloth to a temperature in the region of 700° F. for about two hours. 95
- 25 5. A wide-mesh woven wire cloth of mesh less than 12, the strands of which are held together solely by reason of their weaving, said strands being less than .02 of an inch in diameter, having 100

30

ELMER D. REYNOLDS.

105

35

110

40

115

45

120

50

125

55

130

60

135

65

140

70

145

75

150